

# UNITED STATES PATENT OFFICE.

GONZALO JOSE BUSTAMANTE, OF SOUTH HADLEY, MASSACHUSETTS.

## PRODUCTION OF CELLULOSE FROM VEGETABLE MATTER.

1,402,210.

Specification of Letters Patent.

Patented Jan. 3, 1922.

No Drawing.

Application filed July 26, 1920. Serial No. 398,980.

To all whom it may concern:

Be it known that I, GONZALO JOSE BUSTAMANTE, a subject of the King of Spain, and resident of South Hadley, in the county of 5 Hampshire and State of Massachusetts, have invented certain new and useful Improvements in the Production of Cellulose from Vegetable Matter, of which the following is a specification.

10 It is generally known that cellulose obtained from vegetable matter such as lichens, trees, plants and shrubs of various kinds is capable of offering a certain amount of resistance to the destructive action of heat, 15 pressure, acids and other natural agencies of like character. Theoretically, this power of resistance is unlimited; but practical experiments have proven that there is a definite limit, and that not only is the cellulose 20 decomposed but a very considerable part thereof is lost.

The present invention relates to a cold chemical treatment without pressure, which permits separation of the cellulose from all 25 vegetable matter, impurities and other substances surrounding it. Consideration is taken of the fact that the practical capacity for resistance is limited to a marked degree and, hence, only such materials are used as 30 are favorable to the resistance of the cellulose of the vegetable matter treated, do not deprive it of any of its specific properties, and prevent appreciable loss.

In carrying out the present process, the 35 plants, leaves or stems, or leaves and stems, according to their type, are harvested and then are suitably dried.

The thus prepared vegetable material is then immersed in cold water and separated 40 into coarse fibres in order to facilitate the subsequent penetration by osmosis of the liquid of the treatment bath, this bath being preferably prepared as follows:

Anhydrous lime in great quantity is 45 placed on the floor of a container intended for the treatment, and is covered with the vegetable fibres to a desired height. A cold alkaline solution of 2 to 4° Bé. is supplied thereto in the form of a shower, and there- 50 after a certain amount of volatile alkali, preferably ammonia, which may be of 2% strength, is supplied to the surface of the bath in the form of a shower or in any other form by any desired means. When the ac- 55 tivity of the bath reaches its height, the bath is acidulated gradually with hydrochloric

acid in ratio of 2:1000, and then with sulfuric acid in ratio of 1:1000.

After this bath, to the action of which the material may be subjected, for example, for 60 six hours, the fibrous material is thoroughly washed with cold water and is then placed in a fibre press or mill or subjected to the action of other suitable comminuting mechanism. According to its character, the vegetable material may be placed in a fresh bath of the same character as the previous one, but to which a bleaching agent suited to the vegetable matter under treatment has been added immediately before the introduction 65 of the ammonia or other volatile alkali.

Subsequent baths, similar to those mentioned for the preliminary treatment, may be used according to the degree of comminution of the fibres. 75

After the more or less great time of treatment in the bath, energetic washing with cold water may be carried out for a certain length of time by means of suitable mechanical devices, and the fibres thus obtained 80 may be bleached and refined as considered advisable.

According to this method of treatment, cellulose fibres are obtained which are completely separated from vegetable matter, impurities and other surrounding substances, 85 so that they are suitable for industrial use, either without bleaching or after bleaching and further refinement. The cellulose thus obtained has properties which will compete 90 with those of the best grades of cellulose.

I claim as my invention:

1. The process of obtaining cellulose from vegetable matter, which consists in immersing the vegetable matter to be treated in 95 cold water; separating it into coarse fibres; depositing the fibres in a receptacle containing anhydrous lime; successively supplying a cold alkaline solution and a solution of volatile alkali to said receptacle; successively acidulating the bath thus formed with hydrochloric and sulfuric acids; thereafter washing the fibres with cold water; and finally comminuting said fibres. 100

2. The process of obtaining cellulose from 105 vegetable matter, which consists in immersing the vegetable matter to be treated in cold water; separating it into coarse fibres; subjecting the fibres to the action of a bath comprising anhydrous lime, a cold alkaline solution and a solution of volatile alkali; acidulating said bath; thereafter washing the 110

fibres with cold water; and finally comminuting said fibres.

3. A process according to claim 2 in which a bleach agent is added to the bath before 5 the volatile alkali solution.

4. The process of obtaining cellulose from vegetable matter, which consists in drying the vegetable matter to be treated; immersing it in cold water; separating it into coarse

fibres; depositing the fibres in a receptacle 10 containing anhydrous lime; successively supplying a cold alkaline solution, a bleaching agent and a solution of volatile alkali to said receptacle; acidulating the bath thus formed; thereafter washing the fibres; and 15 finally comminuting said fibres.

In testimony whereof I affix my signature.

G. J. BUSTAMANTE.